

# UNITED STATES PATENT OFFICE.

JOHANNES M. KESSLER, OF WEST ORANGE, NEW JERSEY, ASSIGNOR TO THE  
ARLINGTON COMPANY, OF ARLINGTON, NEW JERSEY, A CORPORATION OF  
NEW JERSEY.

## SOLIDIFIED FUEL.

1,329,610.

Specification of Letters Patent.

Patented Feb. 3, 1920.

No Drawing.

Application filed October 28, 1916. Serial No. 128,181.

To all whom it may concern:

Be it known that I, JOHANNES M. KESSLER, of West Orange, in the county of Essex, and in the State of New Jersey, have invented a certain new and useful Improvement 5 in Solidified Fuel, and do hereby declare that the following is a full, clear, and exact description thereof.

My invention relates to a process of gelatinizing liquids or rendering them more viscous and the product thereof, but particularly in order to produce compositions designed to be used as solidified fuels.

The object of my invention is to provide 10 a process by reason of which liquids containing nitrocellulose may be gelatinized or rendered more viscous as well as the product thereof and, particularly to provide a composition of this character which maintains a supply of a liquid fuel in a solid form both 15 when ignited and when not ignited by reason of the composition of which the fuel forms a part, or so that it will not run out of the container in which it is located, if 20 overturned. Another object is to gelatinize or render more viscous a liquid containing nitrocellulose by the addition of a metal.

Other objects of my invention will appear 25 from the detailed description thereof set forth hereinafter.

While my invention is capable of embodiment in many different forms for the purpose of illustration I shall describe only certain forms thereof hereinafter.

30 For example, the composition made in accordance with my invention may be comprised of—

Nitrocellulose 2 to 10 parts, alcohol 95 parts; and bronze or copper powder .1 part. 35 Preferably the nitrocellulose is present in the proportion of about 5 parts. For the nitrocellulose I may use, if desired celluloid scrap. The alcohol may, for example, be comprised of denatured grain alcohol 90% 40 and wood alcohol 10%. Instead of the bronze or copper powder, I may use other metallic powders provided they have the property of gelatinizing the composition as above pointed out. The composition above 45 referred to when ignited provides a convenient source of heat through the burning of the alcohol which is rendered readily available as the composition is in the form of a stiff paste or jelly, while the alcohol is burning. The characteristics of the composition 50

are such, however, that although the alcohol is rendered readily available after it has become once ignited, at the same time the composition is so stiff after ignition that in case the container which carries the composition 55 is overturned, the contents will not run out.

While I have described my invention in detail, I wish it to be understood that many changes may be made therein, without departing from the spirit of my invention. 65

I claim:

1. A solidified liquid fuel composition containing nitrocellulose, and a metallic powder.

2. A solidified liquid fuel composition 70 containing nitro-cellulose, and a metallic powder containing copper.

3. A solidified liquid fuel composition containing nitro-cellulose, and bronze powder.

4. A solidified liquid fuel composition containing nitro-cellulose, a metallic powder, and alcohol.

5. A solidified liquid fuel composition containing nitro-cellulose, a metallic powder 80 containing copper, and alcohol.

6. A solidified liquid fuel composition containing nitro-cellulose, bronze powder, and alcohol.

7. A solidified liquid fuel composition 85 containing nitro-cellulose, a metallic powder, and alcohol, in the proportion of 5 parts of nitro-cellulose, 95 parts alcohol and 0.1 part metallic powder.

8. A solidified liquid fuel composition 90 containing nitro-cellulose, a metallic powder containing copper, and alcohol, in the proportion of 5 parts of nitro-cellulose, 95 parts alcohol and 0.1 part metallic powder.

9. A solidified liquid fuel composition 95 containing nitro-cellulose, bronze powder, and alcohol, in the proportion of 5 parts of nitro-cellulose, 95 parts alcohol and 0.1 part metallic powder.

10. A process of solidifying a liquid fuel 100 which comprises gelatinizing a solution containing nitrocellulose dissolved in more than three times its weight of alcohol, by treatment with a pulverized metal.

11. A process of solidifying a liquid fuel 105 which comprises gelatinizing a solution, containing nitrocellulose dissolved in more than three times its weight of alcohol, by treatment with a pulverized substance containing metallic copper.

- 2
12. A process of solidifying a liquid fuel which comprises gelatinizing a solution, containing nitrocellulose dissolved in more than three times its weight of alcohol, by treatment with bronze powder.
13. A process of solidifying a liquid fuel which comprises gelatinizing a solution, containing an aliphatic alcohol and nitrocellulose in the proportion of less than 10% of the alcohol by treatment with a pulverized metal.
14. A process of solidifying a liquid fuel which comprises gelatinizing a solution, containing a relatively small proportion of nitrocellulose dissolved in a mixture of ethyl and methyl alcohols, by treatment with a pulverized metal.
15. A process of solidifying a liquid fuel which comprises gelatinizing a solution, containing a relatively small proportion of nitrocellulose dissolved in a mixture of ethyl and methyl alcohols, by treatment with a pulverized substance containing metallic copper.
16. A process of solidifying a liquid fuel which comprises gelatinizing a solution, containing a relatively small proportion of nitrocellulose dissolved in a mixture of ethyl and methyl alcohols, by treatment with bronze powder.
17. A process of solidifying a liquid fuel which comprises gelatinizing a solution, containing a relatively small proportion of nitrocellulose dissolved in a mixture of ethyl and methyl alcohols in the proportion of approximately 10 to 1, by treatment with a pulverized metal.
18. A process of solidifying a liquid fuel which comprises gelatinizing a solution containing 5 to 10 parts nitrocellulose dissolved in 90 to 95% of alcohol, by treatment with one-tenth part of bronze powder.
19. A process of solidifying a liquid fuel which comprises gelatinizing a solution of nitrocellulose in an organic aliphatic compound, by treatment with a bronze powder in approximately the proportion of 0.1% of the solution.
20. A process of solidifying a liquid fuel which comprises gelatinizing a solution of nitrocellulose in a proportion of less than 10% of the weight of the fuel by treatment with a pulverized metal.

In testimony that I claim the foregoing I have hereunto set my hand.

JOHANNES M. KESSLER.

Witnesses:

PETER J. NAHER,  
JOHN H. CLEWELL, Jr.